

## UNITED STATES PATENT OFFICE

2,335,017

## LUBRICATING COMPOSITION

John G. McNab, Cranford, and Carroll J. Wilson  
and Carl Winning, Westfield, N. J., assignors to  
Standard Oil Development Company, a corpora-  
tion of Delaware

No Drawing. Application December 31, 1941,  
Serial No. 425,128

17 Claims. (CL 252—48)

This invention relates to lubricating oils and methods of preparing the same, and more particularly to mineral lubricating oil compositions for use as crankcase lubricants in internal combustion engines.

Because in recent years the requirements for lubricating oils for gasoline and Diesel engines have steadily been made more stringent, it has been proposed to add various ingredients to these oils to improve their behavior in such service. One purpose of these ingredients is to impart detergency to the oils, thus bringing about greater engine cleanliness and avoiding ring sticking, carbon formation and varnish deposition. Certain of these ingredients also impart oxidation resistant properties to oils, thereby tending to inhibit the development of corrosive ingredients in such oils. Corrosion-preventing addition agents are particularly required when the oil is to come in contact with the newer type of alloys of silver and cadmium and of copper and lead, which are now widely used as bearing metals.

Various metal-containing organic compounds which also contain sulfur in a lower state of oxidation have been found particularly useful as detergents as well as corrosion-preventing agents. Such compounds include metallic thiophenolates and thioxanthates, metallic derivatives of various phenol sulfides and disulfides, etc. In use, the effectiveness of these compounds is gradually spent. The detergent capacity becomes exhausted as deterioration products, soot, dirt, varnish, etc., accumulate in the lubricant and saturate the adsorptive power of the additive. In engines equipped with a filter, the latter tends to remove the additive, particularly when the additive is adsorbed on contamination products which are strained out by the filter. The oxidation processes which are underway in an oil during use operate upon the antioxidant functions of the additive and thus also contribute to its exhaustion. The oxidation of the oil also creates insoluble substances which the detergent is called upon to adsorb, thus lessening its capacity for dispersing contamination products which enter the oil, and acidic substances are also formed which may react directly with the detergent to destroy its efficacy. When the detergent is employed also to impart corrosion resistant properties to the oil, the above degradation phenomena all hasten to break down this corrosion resistance.

It is apparent from the foregoing observations that any auxiliary agent capable of stabilizing the oil in the presence of the detergent should materially extend the benefits obtained with the latter. It should also afford protection against corrosion after the detergent has become saturated with dispersed materials or removed by an oil filter. However, the expected additional

benefits are not realized when certain well-known corrosion inhibitors and stabilizing agents, such as sulfurized sperm oil, dibenzyl disulfide, triamylphenyl phosphite and the like, are added to the oil containing a metallic detergent agent. In some cases, in fact, the corrosive effect is even increased by adding such compounds.

It has now been found, in accordance with the present invention, that very satisfactory results may be secured by adding to the oil, in addition to the metallic sulfur compound, a tertiary aliphatic ether of a phenol, this compound being more particularly defined in the description which follows. This combination of addition agents provides for detergent action in the early stages of the use of the oil, as well as continued corrosion inhibiting effect after the metallic detergent compound has been removed to some degree by the filter, and whether a filter is or is not used there is a distinct advantage in using the combination of additives here described, since the corrosion of metal surfaces and the formation of deposits on engine parts are notably reduced.

The addition agent which is to serve, in accordance with this invention, as the detergent agent as well as a corrosion preventing agent in the early stages of use, may be defined as an organic compound containing a metal or a basic radical, such as ammonium, sulfonium or phosphonium, etc., and containing also at least one atom of sulfur in divalent form. There may be more than one atom of sulfur in the molecule, but at least one atom of sulfur is divalent and is linked either directly to carbon or to another sulfur atom which in turn is linked directly to carbon. This class of metal-containing sulfur compounds includes metallic derivatives of such organic compounds as the mercaptides, thiophenolates, xanthates, thioxanthates, metallic derivatives of various sulfides and disulfides of phenols, etc. This class of addition agents also includes the corresponding compounds in which sulfur is replaced by selenium or tellurium.

Typical general classes of metal sulfur compounds included within the above definition are the following:

A. Compounds in which a metal is attached to sulfur

1. Metallic thioalcoholates or mercaptides

R-SM

2. Metallic thiophenolates



## 3. Metal salts of thiocarboxylic acids



## 4. Metallic xanthates



## 5. Metallic thioxanthates



## 6. Metallic thiocarbonates other than xanthates



## 7. Metallic thiocarbamates



## 8. Metallic dithiocarbamates



## B. Sulfur compounds in which a metal is attached to elements other than sulfur

## 1. Metallo-organic compounds



## 2. Metallic soaps



## 3. Metallic derivatives of thioethers



In any of the above formulas, whenever the metal is other than monovalent, the other valences may be satisfied by the same group or by different groups, as, for example, in the following:



In all of the above formulas R, R', etc., represent aliphatic or aromatic radicals and M, M', etc., represent metals or other basic acting units, such as basic radicals. If desired, S may be replaced by Se or Te.

In any of the various types of sulfur compounds named above any of the aromatic or aliphatic radicals may contain further substituent atoms or groups, such as oxygen, sulfur, halogen, 10 nitrogen or phosphorus atoms, as well as groups such as alkyl, aralkyl, aryl, cycloalkyl, -OH, -SH, -NH<sub>2</sub>, -NH (alkyl), -N (alkyl)<sub>2</sub>, -O (alkyl), -O (aryl), -S (alkyl), -S (aryl), -CO (alkyl), -CO (aryl), -CHO, and -COO (alkyl).

A preferred group of compounds for use in the present invention is that containing the radical defined by the formula



in which M is a metal or a basic radical, X is oxygen or sulfur which is attached to a carbon atom which is in turn attached only to hydrogen and/or other carbon atoms. In the above formula R is an aliphatic or aromatic radical and n is an integer, 1 to 4.

A particularly preferred group of compounds are the metal salts of phenolic thioethers



in which M is a metal, X is oxygen or sulfur, Ar is an aromatic nucleus, R is an organic group, 35 S is sulfur and n is an integer, 1 to 4. Ar may represent a single benzene ring or a condensed ring system and the substituents R may be alkyl, aryl, aralkyl, alkaryl, or substituted groups and may occur more than once in each ring. The 40 group S<sub>n</sub> may have any of the following configurations:

(1) -S-, -S-S-, -S-S-S-, etc.

(2) -S-

(3) -S-S-S-

50 (4) -S-



55 The radicals represented by R in the above formula should be of sufficient size to impart adequate oil solubility to the compounds and such alkyl radicals as butyl, amyl, diisobutyl, decyl, cetyl, and stearyl have been found satisfactory.

60 Whenever the diisobutyl group is mentioned in this specification, the tetramethylbutyl radical, formed by polymerizing isobutylene, is meant.

When the phenolic groups are alkylated with petroleum olefinic hydrocarbons, such as refined 65 gases and the like, the resulting products may comprise a mixture of compounds with different sizes of alkyl groups. Mixtures of metal-containing sulfur compounds prepared from such mixed alkyl groups are also contemplated in this invention.

In some cases the phenolic compounds may be alkylated with long chain groups such as those derived from petroleum wax or an ester wax. In such cases one wax group may be attached to each 75 aryl group or several aryl groups may be attached

to one wax group at several points along the chain, as represented below.



It should be understood, of course, that these are merely examples of the types of compounds which can be formed during alkylation and that the invention is not to be limited by this description.

Among the compounds falling in the preferred class those most frequently used are the sulfides or disulfides of metallic derivatives of phenols, for example, barium bis-(diisobutyl phenoxy) sulfide, magnesium bis(tertiary amyl phenoxy) sulfide, and the various metallic salts of alkylated hydroxybenzyl sulfide and alkylated bis(hydroxybenzyl) disulfide.

The metals of the above described class of compounds may be selected from any of the metallic groups, but are preferably members of groups I, II, III, IV or VIII of the periodic table. Particularly desirable are group II metals, barium, calcium, magnesium, and zinc, and, in addition, cobalt, nickel, and tin. In place of the metals there may be substituted any of the well-known basic radicals, such as ammonium or the various onium groups, such as the quaternary ammonium base radicals and the corresponding sulfonium, phosphonium, arsonium or pyridonium radicals and the like.

These compounds may be prepared by any well-known methods. For example, barium bis-(diisobutyl phenoxy) sulfide may be prepared by alkylating phenol with diisobutylene, followed by treatment with sulfur chloride to form the thioether and finally saponification with barium hydroxide to form the salt. The invention is not to be limited by any method of preparing these additives, however.

The following is a description of one method which has been used for preparing barium bis-(diisobutyl phenoxy) sulfide (barium salt of diisobutyl hydroxy phenyl sulfide).

#### EXAMPLE 1

A 31% solution of diisobutyl phenol in chloroform, containing a total of 217 lbs. of diisobutyl phenol, was placed in a reaction vessel. Over a period of 3 hours 80.6 lbs. of sulfur chloride,  $SCl_2$ , were added gradually, the temperature of the mixture being held at 20-25° C. Following this step, the mixture was heated under reflux for two hours and the chloroform then removed by heating to 100° C. Finally, the product was blown with carbon dioxide for several hours until neutral to Congo red paper.

The amount of diisobutyl hydroxy phenyl sulfide present in the reactor after the above procedure was estimated to be 238 pounds. About 395 lbs. of an extracted Mid-Continent lubricating oil (about 52 secs. viscosity (Saybolt) at 210° F.) were pumped into the reactor and mixed with the diisobutyl hydroxy phenyl sulfide. While agitation was continued, the temperature was raised to 210° F. and a stream of nitrogen under 2 lbs./sq. in. pressure was blown in at the bottom of the reactor. Then 75 lbs. of stearyl alcohol were added and the temperature raised to 230° F. Gradual addition of 185 lbs. of a technical grade of barium hydroxide octahydrate,



was then begun, the temperature first being raised to 240° F. and the stream of nitrogen continued.

After about 85% (163 lbs.) of the barium hydroxide had been added (requiring about 6 hours) excessive foaming occurred, but it was found that this could be controlled by raising the temperature to 250° F., whereupon the balance of the barium hydroxide was added. Following this, the batch was blown with nitrogen for one hour at 230° F. to remove all water. Four pounds of "Hyflow" filter aid were added and the mixture filtered at 260° F., yielding a concentrate of oil containing 40% of the barium salt of diisobutyl hydroxy phenyl sulfide and 10% of stearyl alcohol. Analysis indicated 9.02% barium, almost exactly the theoretical amount for a 40% solution of the barium salt of diisobutyl hydroxy phenyl sulfide,  $Ba(O-C_6H_5-C_8H_{17})_2S$ .

The second addition agent, to be added to the lubricating oil base in addition to a metallic-sulfur compound of the above described class, may be defined as an organic compound of the formula



where  $Ar$  is an aromatic nucleus, which may contain one or more benzene rings or a condensed ring system such as naphthalene and the like,  $R$  is an organic radical,  $R'$  is a tertiary aliphatic radical, and  $n$  is an integer indicating the number of radicals  $R$  which are attached to the nucleus. The  $R$  groups may be alike or different. The substituent group or groups  $R$  appear to be required to activate the ether group and enable the compound to perform its function. Included within the scope of the above formula are compounds in which one or more of the hydrogen atoms of the aromatic nucleus or of the radicals  $R$  and  $R'$  may be replaced by substituent atoms, such as oxygen, sulfur, nitrogen, phosphorus or halogen, or groups, such as alkyl, aralkyl, cycloalkyl,  $-OH$ ,  $-SH$ ,  $-NH_2$ ,  $-NH(alkyl)$ ,  $-N(alkyl)_2$ ,  $-O(alkyl)$ ,  $-CO(aryl)$ ,  $-S(alkyl)$ ,  $-S(aryl)$ ,  $-CO(alkyl)$ ,  $-CO(aryl)$ ,  $-CHO$ ,  $-COOH$ ,  $-COO(alkyl)$ , as well as groups containing metals, such as  $-OM$ ,  $-SM$ ,  $-COOM$ ,  $-CSSM$ , etc., or, in place of the metals, basic groups, such as the ammonium, sulfonium, phosphonium, and pyridonium base radicals.  $M$  represents a metal equivalent.

A more preferred group of compounds, falling within the class defined immediately above, are those having a benzene ring as the aromatic nucleus. Especially suitable are the compounds defined by the formula



in which  $R$  and  $R'$  are aliphatic radicals or hydrogen and  $R''$  is a tertiary aliphatic radical. An example of such a compound is the tertiary butyl ether of ortho tertiary butyl p-cresol.

Among other ethers which may be employed in this invention are the tertiary butyl ether of ortho tertiary butyl para isopropyl phenol, tertiary amyl ether of ortho tertiary amyl para isopropyl phenol, tertiary hexyl ether of ortho tertiary hexyl para isopropyl phenol, tertiary butyl ether of ortho tertiary butyl para isobutyl phenol, tertiary butyl ether of ortho tertiary butyl para ethyl phenol, tertiary butyl ether of ortho tertiary butyl para normal hexyl phenol, tertiary butyl ether of

ortho secondary butyl para cresol, tertiary butyl ether of ortho normal butyl para cresol, tertiary butyl ether of ortho secondary amyl para cresol, tertiary butyl ether of ortho secondary butyl para ethyl phenol, tertiary butyl ether of ortho secondary butyl para normal butyl phenol, tertiary butyl ether of ortho secondary butyl para isobutyl phenol, tertiary butyl ether of ortho normal butyl para hexyl phenol, tertiary amyl ether of ortho secondary butyl para isobutyl phenol, tertiary butyl ether of ortho secondary amyl para isobutyl phenol, tertiary butyl ether of 4-tertiary butyl alpha-naphthol tertiary amyl ether of 2-phenyl-4-isobutyl phenol, tertiary butyl ether of 2,6-di(propylamino)-4-methyl phenol, tertiary butyl ether of ortho chlorohexyl para cresol, tertiary amyl ether of ortho tertiary amyl para cresol sulfide, tertiary butyl ether of 2-butyl-4-ethyl-6-chlorophenol, and tertiary hexyl ether of 2-decyl-4-ethyl resorcinol.

A still further class of ethers which may be advantageously employed are those having long side chain groups, such as those derived from petroleum wax or an ester wax. In such cases one wax group may be attached to each aryl group or several aryl groups may be attached to one wax group at several points along the chain. For example, when long chain alkyl groups are introduced into the compounds, as by alkylation with halogenated paraffin wax, mono-halogenated wax tends to give alkylated phenyl ethers of the following types:

(a)



(b)



in which R is a tertiary aliphatic radical, R' is hydrogen or an aliphatic radical, and m and n are integers. However, if poly-halogenated wax is used, it is possible for two or more phenyl ether groups to be attached to the same alkyl chain as follows:



The above described tertiary aliphatic ethers of phenols may conveniently be prepared by reacting a phenol with a tertiary olefin, e. g., isobutene, or with a tertiary aliphatic alcohol, e. g., tertiary butyl alcohol, in the presence of a catalyst such as sulfuric acid. In general, the temperature should be above that of the phenol being reacted. A satisfactory method for the preparation of the tertiary butyl ether of ortho tertiary butyl p-cresol, one of the preferred additives, is as follows: p-Cresol is mixed with about 5% of its weight of 96% commercial sulfuric acid and agitated at about 70° C. while isobutene is bubbled through the mixture. After completion of the reaction, as indicated by the flow of isobutene from the gas exit, the reaction mixture is blown with steam and washed with hot water and dilute alkali until neutral. A high yield of an oily material is obtained, which readily crys-

tallizes on cooling. The product may be recrystallized from hot alcohol. The same product may be obtained by reacting p-cresol with tertiary butyl alcohol. In this case the amount of

5 sulfuric acid catalyst is preferably quite large, i. e., of the order of one mol of catalyst per mol of p-cresol. Temperatures from about 0° to about 50° C. may be used, preferably from 25° to 40° C.

10 The lubricating oil base stocks of this invention may be straight mineral lubricating oils or distillates derived from paraffinic, naphthenic, asphaltic or mixed base crudes, or, if desired, various blended oils may be employed as well as

15 residuals, particularly those from which asphaltic constituents have been carefully removed. The oils may be refined by conventional methods using acid, alkali and/or clay or other agents, such as aluminum chloride, or they may be extracted oils

20 produced, for example, by solvent extraction with solvents of the type of phenol, sulfur dioxide, furfural, dichloro ethyl ether, propane, nitrobenzene, crotonaldehyde, etc. Hydrogenated oils or white oils may be employed as well as synthetic oils prepared, for example, by the polymerization of olefins or by the reaction of oxides of carbon with hydrogen or by the hydrogenation of coal or its products. In certain instances

25 cracking coal tar fractions and coal tar or shale oil distillates may also be used. Also, for special applications, animal, vegetable or fish oils or their hydrogenated or volatilized products may be employed, either alone or in admixture with mineral oils.

30 35 For the best results, however, the base stock chosen should usually be that oil which without the additive present gives the optimum performance in the service contemplated. Since one advantage of the additives is that their use also

40 makes feasible the employment of less satisfactory mineral oils or other oils, no strict rule can be laid down for the choice of the base stock. Certain essentials must of course be observed. The oil must possess the viscosity and volatility

45 characteristics known to be required for the service contemplated. The oil must be a satisfactory solvent for the additive, although in some cases auxiliary solvent agents may be used. The lubricating oils, however they may have been produced,

50 may vary considerably in viscosity and other properties depending upon the particular use for which they are desired, but they usually range from about 40 to 150 seconds Saybolt viscosity at 210° F. For the lubrication of medium

55 and high speed Diesel engines the general practice has been to use a lubricating oil base stock prepared from naphthenic or aromatic crudes and having a Saybolt viscosity at 210° F. of 45 to 90 seconds and a viscosity index of 0 to 50. However, in certain types of Diesel service, and in gasoline engine service, oils of higher viscosity

60 index are often required, for example, up to 75 or 100, or even higher, viscosity index.

In addition to the materials to be added according to the present invention, other agents may also be used such as dyes, pour depressors, heat thickened fatty oils, sulfurized fatty oils, organo metallic compounds, metallic or other soaps, sludge dispersers, antioxidants, thickeners, viscosity index improvers, oiliness agents, resins, rubber, olefin polymers, volatilized fats, volatilized mineral oils, and/or volatilized waxes and colloidal solids such as graphite or zinc oxide, etc. Solvents and assisting agents, such as esters, ketones, alcohols, aldehydes, halogenated or ni-

trated compounds, and the like, may also be employed.

Assisting agents which are particularly desirable are the higher alcohols having 8 or more carbon atoms and preferably 12 to 20 carbon atoms. The alcohols may be saturated straight and branched chain aliphatic alcohols such as octyl alcohol,  $C_8H_{17}OH$ , lauryl alcohol,  $C_{12}H_{25}OH$ , cetyl alcohol,  $C_{16}H_{33}OH$ , stearyl alcohol, sometimes referred to as octadecyl alcohol,  $C_{18}H_{37}OH$ , and the like; the corresponding olefinic alcohols such as oleyl alcohol; cyclic alcohols, such as naphthenic alcohols; and aryl substituted alkyl alcohols, for instance, phenyl octyl alcohol, or octadecyl benzyl alcohol or mixtures of these various alcohols, which may be pure or substantially pure synthetic alcohols. One may also use mixed naturally occurring alcohols such as those found in wool fat (which is known to contain a substantial percentage of alcohols having about 16 to 18 carbon atoms) and in sperm oil (which contains a high percentage of cetyl alcohol); and although it is preferable to isolate the alcohols from those materials, for some purposes the wool fat, sperm oil or other natural products rich in alcohols may be used per se. Products prepared synthetically by chemical processes may also be used, such as alcohols prepared by the oxidation of petroleum hydrocarbons, e. g., paraffin wax, petrolatum, etc.

Generally the amount of each of the additives of the present invention in the finished lubricant composition should be between the approximate limits of 0.02 and 2.0%, and preferably between 0.1 and 1.0%, the exact amount to be used depending to a certain extent on the particular compounds used, the character of the oil base and the operating conditions of the engine in which the lubricant is to be used.

Typical examples of additive mixtures which may be employed in practicing this invention include the following: the tertiary butyl ether of ortho secondary amyl p-cresol with calcium tertiary amyl thiophenolate; the tertiary butyl ether of ortho tertiary butyl p-cresol with zinc lauryl mercaptide; the tertiary butyl ether of ortho tertiary butyl p-isopropyl phenol with tin dicyclohexyl dithiocarbamate; the tertiary butyl ether of ortho secondary butyl p-ethyl phenol with the barium salt of wax-alkylated phenoxy thioether; the tertiary hexyl ether of ortho n-butyl p-cresol with nickel amyl xanthate, the tertiary butyl ether of ortho tertiary butyl p-cresol with the barium salt of bis-(dibutyl phenoxy) sulfide; and the tertiary amyl ether of ortho n-butyl p-cresol with the aluminum salt of thiooleic acid. Compositions in which two or more metal compounds are used with one or more ethers or in which one metal compound is used with two or more ethers are also contemplated in this invention. The effects of some of these additive mixtures on the corrosion resistance and engine performance of oils in which they were blended are shown in the examples given below.

The first two of the following examples show the effect of the use of a tertiary aliphatic ether of an aromatic compound upon the corrosion of copper-lead bearings when used in combination with a metal-containing sulfur compound in a lubricating oil, as compared with the use of several known corrosion inhibitors in combination with the same metallic sulfur compounds. In these examples the well-known corrosion inhibi-

tors had only an adverse effect on the corrosive properties of the oil, while the ether compound aided considerably in preventing corrosion.

#### EXAMPLE 2

Samples of oil blends containing, separately, well-known corrosion inhibitors as well as a tertiary aliphatic ether of the present invention, in addition to one or more of the metal-containing sulfur compounds of the present invention, as well as samples of oil containing the same metal sulfur compounds, but with the omission of the second corrosion inhibitor, were submitted to a bearing corrosion test in which the extent of weight loss of alloy bearings, due to corrosion by the oils, was determined. This test was conducted as follows:

500 cc. of the oil were placed in a glass oxidation tube (13" long and 2 $\frac{1}{8}$ " diameter) fitted at the bottom with a  $\frac{1}{4}$ " bore air inlet tube perforated to facilitate air distribution. The oxidation tube was then immersed in a heating bath so that the oil temperature was maintained at 325° F. during the test. Two quarter sections of 25 automotive bearings of copper-lead alloy of known weight and having an area of 50 sq. cm. were attached on opposite sides of a stainless steel rod which was then immersed in the test oil and rotated at 600 R. P. M., thus providing 30 sufficient agitation of the sample during the test. Air was then blown through the oil at the rate of 2 cubic feet per hour. At the end of each hour fresh bearings were supplied and 15% of the oil in the oxidation tube was removed and a corresponding amount of fresh oil was added. After 35 the bearings were removed in each test, they were washed with naphtha and weighed to determine the amount of bearing weight lost by corrosion. The tests were continued in each case until the 40 cumulative weight loss of all the bearings tested with a given oil blend was 50 milligrams.

A refined lubricating oil of S. A. E. 20 grade and consisting of an extracted Mid-Continent paraffinic oil was blended with 0.5% of barium bis-(dibutyl phenoxy) sulfide, 0.5% of barium bis-(dibutyl phenoxy) disulfide and 0.25% of stearyl alcohol. A sample of this blend was submitted to the above described test, as well as samples of the same blended, respectively, with 45 1% of sulfurized polymer oil, 1% of sulfurized sperm oil, 0.25% of dibenzyl disulfide, and 0.5% of the tertiary butyl ether of ortho tertiary butyl p-cresol. (Polymer oil as used in these examples comprises synthetic oils falling in the lubricating oil range prepared by polymerization of isobutylene with boron fluoride.) The results are shown 50 in Table I, in which the "bearing life" refers to the number of hours which elapsed to produce a cumulative bearing weight loss of 50 milligrams.

Table I

|     | Oil                                                                                                                              | Bearing life |
|-----|----------------------------------------------------------------------------------------------------------------------------------|--------------|
| (A) | Base oil + 0.5% barium bis-(dibutyl phenoxy) sulfide<br>+ 0.5% barium bis-(dibutyl phenoxy) disulfide<br>+ 0.25% stearyl alcohol | Hours<br>8.2 |
| (B) | Oil A + 1.0% sulfurized polymer oil                                                                                              | 7.0          |
| (C) | Oil A + 1.0% sulfurized sperm oil                                                                                                | 6.1          |
| (D) | Oil A + 0.25% dibenzyl disulfide                                                                                                 | 5.0          |
| (E) | Oil A + 0.5% tert.-butyl ether of ortho tert.-butyl p-cresol                                                                     | 17.5         |

The results given in Table I clearly show that 75 the various sulfur compounds commonly advo-

cated as inhibitors of corrosion actually increased corrosiveness when used in the compounded lubricant, whereas the tertiary butyl ether of the present invention markedly decreased the corrosiveness and actually more than doubled the bearing life of the oil.

#### EXAMPLE 3

In this example, a refined mineral lubricating

bination of addition agents which constitutes the present invention.

#### EXAMPLE 4

5 Samples of a base oil of S. A. E. 30 grade, alone and mixed with one or more of the additives of the present invention, were submitted to the corrosion test described in Example 2, using copper-lead bearings as before and the results are shown in Table III.

Table III

| Oil                                                                                                                                  | Cumulative bearing weight loss, milligrams |                 |                 |                 |                 |                 |                 |                 |                  |                  |                  |  |
|--------------------------------------------------------------------------------------------------------------------------------------|--------------------------------------------|-----------------|-----------------|-----------------|-----------------|-----------------|-----------------|-----------------|------------------|------------------|------------------|--|
|                                                                                                                                      | 1 hour of test                             | 2 hours of test | 3 hours of test | 4 hours of test | 5 hours of test | 6 hours of test | 7 hours of test | 8 hours of test | 12 hours of test | 16 hours of test | 24 hours of test |  |
| (A) Refined mineral oil (S. A. E. 30)                                                                                                | 4                                          | 8               | 24              | 47              | 85              | 136             | 200             | —               | —                | —                | —                |  |
| (B) Oil A + 0.32% barium bis-(diisobutyl phenoxy) sulfide + 0.32% barium bis-(diisobutyl phenoxy) disulfide + 0.163% stearyl alcohol | 2                                          | 4               | 5               | 8               | 12              | 15              | 19              | 24              | 32               | 155              | —                |  |
| (C) Oil A + 0.25% tert.-butyl ether of ortho tert.-butyl p-cresol                                                                    | 2                                          | 4               | 6               | 8               | 10              | 13              | 18              | 23              | 31               | 180              | —                |  |
| (D) Oil B + 0.25% tert.-butyl ether of ortho tert.-butyl p-cresol                                                                    | 4                                          | 6               | 8               | 11              | 13              | 15              | 19              | 23              | 30               | 42               | 73               |  |

oil base of S. A. E. 30 grade, consisting of 35% of extracted Coastal oil and 65% of paraffinic oil, was blended with 0.25% of barium bis-(diisobutyl phenoxy) sulfide, 0.25% of barium bis-(diisobutyl phenoxy) disulfide and 0.125% of stearyl alcohol. Samples of this blend alone and with the addition of 0.25% of triphenyl phosphite were each submitted to a test similar to that described in Example 2. The results are shown in Table II, in which the actual cumulative loss in bearing weight at the end of each second hour during the test is recorded.

These data show that the corrosiveness of the mineral oil is somewhat reduced by adding the barium salts of bis-(diisobutyl phenoxy) sulfide and disulfide plus stearyl alcohol, the blend taking 16 hours to corrode the bearings as much as the mineral oil alone did in 8 to 7 hours. By adding to this compounded oil a small amount of a tertiary alkyl ether of the present invention the corrosiveness is still further reduced, the weight loss with this oil (oil D) in 24 hours not being as much as in 5 hours with the un compounded oil. On the other hand, if the same amount of ter-

Table II

| Oil                                                                                                                                     | Cumulative bearing weight loss, milligrams |                 |                 |                 |                  |                  |                  |                  |
|-----------------------------------------------------------------------------------------------------------------------------------------|--------------------------------------------|-----------------|-----------------|-----------------|------------------|------------------|------------------|------------------|
|                                                                                                                                         | 2 hours in test                            | 4 hours in test | 6 hours in test | 8 hours in test | 10 hours in test | 12 hours in test | 14 hours in test | 16 hours in test |
| (A) Base oil + 0.25% barium bis-(diisobutyl phenoxy) sulfide + 0.25% barium bis-(diisobutyl phenoxy) disulfide + 0.125% stearyl alcohol | 10                                         | 22              | 41              | 76              | 106              | 161              | 253              | 400              |
| (B) Oil A + 0.25% triphenyl phosphite                                                                                                   | 6                                          | 17              | 45              | 113             | 233              | 346              | —                | —                |

It can be seen that the triphenyl phosphite actually increased the corrosiveness of the compounded oil rather than decreased it, which is surprising in view of the known effect of this additive as a corrosion inhibitor in the absence of sulfur-containing metallic compounds.

In the following series of tests, described as Examples 4, 5, and 6, various oil blends containing, separately or in the same oil, the preferred addition agents of the present invention, were submitted to tests similar to that described in Example 2, the modifications in each case being indicated below. The results shown indicate the advantageous use of the preferred com-

60 tiary alkyl ether is added to the mineral oil without the metallic additives the resulting blend (oil C) is more corrosive than the oil containing no ether but containing the alcohol and metal compounds (oil B).

#### EXAMPLE 5

The oil blends as described in this example were submitted to bearing corrosion tests similar to the test described in Example 2, except that in the present case the bearings were replaced only after four hour intervals and the area of each test bearing was 25 sq. cm. The cumulative weight losses at the end of the various four hour periods are indicated in Table IV:

Table IV

| Oil                                                                  | Cumulative bearing weight loss, milligrams |         |          |          |          |          |          |
|----------------------------------------------------------------------|--------------------------------------------|---------|----------|----------|----------|----------|----------|
|                                                                      | 4 hours                                    | 8 hours | 12 hours | 16 hours | 20 hours | 24 hours | 28 hours |
| (A) Refined mineral lubricating oil (S. A. E. 30)                    | 1                                          | 252     | —        | —        | —        | —        | —        |
| (B) Oil A + 1.0% barium bis-(diisobutyl phenoxy) sulfide             | 2                                          | 4       | 7        | 147      | —        | —        | —        |
| (C) Oil B + 0.25% additive M <sup>1</sup>                            | 2                                          | 5       | 5        | 14       | —        | —        | —        |
| (D) Oil A + 1.0% nickel dicyclohexyl dithiocarbamate                 | 0                                          | 2       | 4        | 6        | 10       | 75       | 15       |
| (E) Oil D + 0.25% additive M <sup>1</sup>                            | 1                                          | 4       | 5        | 7        | 9        | 15       | 18       |
| (F) Oil A + 1.0% barium bis-(diisobutyl hydroxy benzyl amyl) sulfide | 0                                          | 0       | 7        | 29       | 160      | —        | —        |
| (G) Oil F + 0.25% additive M <sup>1</sup>                            | 0                                          | 0       | 1        | 3        | 10       | 105      | —        |

<sup>1</sup> Tertiary butyl ether of ortho tertiary butyl p-cresol.

These data show that although the addition of a metal salt of a sulfur-containing compound in each case reduced the corrosiveness of the uncompounded mineral oil to some extent, a much greater improvement was obtained by adding the tertiary butyl ether of ortho tertiary butyl para-cresol.

**EXAMPLE 6**

Other oil blends were tested in the manner described in Example 2, except that in this case two copper-lead bearing halves and two cadmium-silver bearing halves were placed alternately on opposite sides of the stainless steel rod and immersed in the oil samples as previously described and the tests conducted for five hours. Table V shows the total bearing loss in each case.

Table V

|     | Oil                                                                                                                              | Five hour corrosion test-bearing weight loss, milligrams |                | 20 |
|-----|----------------------------------------------------------------------------------------------------------------------------------|----------------------------------------------------------|----------------|----|
|     |                                                                                                                                  | Copper-lead                                              | Cadmium-silver |    |
| (A) | Conventionally refined Coastal naphthalene oil (55 secs. vis. Saybolt at 210° F.) +0.5% cobalt bis-(tert. amyl phenoxy) sulfide. | 12                                                       | 1              |    |
| (B) | Oil A +0.5% additive M <sup>1</sup>                                                                                              | 2                                                        | 1              |    |

<sup>1</sup> Tertiary butyl ether of ortho tertiary butyl p-cresol.

These data further demonstrate that the ether additive of the present invention inhibits the corrosiveness of compounded oils toward alloy bearings. Similar results were also obtained in a different type of corrosion test as shown in Example 7.

**EXAMPLE 7**

Oil blends were also subjected to the standard Underwood bearing corrosion test, which was conducted as follows:

The polished bearings of the Underwood machine were thoroughly abraded with emery cloth so that corrosion would proceed uniformly and then accurately weighed. The apparatus was filled with 1500 cc. of the lubricant under test and the pump and heater started. The oil pressure was regulated to 10 pounds per square inch by means of by-pass valves and maintained at this pressure throughout the test. As soon as the temperature of the oil reached 275° F. the heater and pump were turned off just long enough to put the already prepared and weighed bearings in place. Two copper-lead and two cadmium-silver bearing halves were used simultaneously in each test. At the end of 20 hours the bearings were removed, cleaned with naphtha, dried and weighed. The weight loss was taken as a measure of the corrosiveness of the oil.

In Table VI are shown the results of tests using the above procedure. The base oil consisted of a conventionally refined Coastal oil having a viscosity of 55 seconds Saybolt at 210° F.

Table VI

|     | Oil                                                     | Bearing weight loss, milligrams |                | 5 |
|-----|---------------------------------------------------------|---------------------------------|----------------|---|
|     |                                                         | Copper-lead                     | Cadmium-silver |   |
| (A) | Base oil +0.5% cobalt bis-(tert. amyl phenoxy) sulfide. | 10                              | 1              |   |
| (B) | Oil A +0.5% additive M <sup>1</sup>                     | 4                               | 1              |   |

<sup>1</sup> Tertiary butyl ether of ortho tertiary butyl p-cresol.

In the examples which follow there are given results of tests of several oil blends run in various engines operating under different degrees of severity. These examples serve further to show the advantages to be gained by using in a lubricating oil a combination of additives illustrating the present invention.

**EXAMPLE 8**

A mineral lubricating oil blend containing metal salts of sulfur compounds as described below and a similar blend containing in addition a tertiary alkyl ether of an alkylated phenol were each tested for 500 hours in a General Motors 3-cylinder Diesel engine. The following engine conditions prevailed in each test: speed, 2000 R. P. M.; power output, 80 brake H. P.; back pressure, 6 in. of mercury; water temperature, 180° F.; oil sump temperature, 230° F.; intake air temperature, 105° F. Results obtained, expressed on a demerit rating system, are shown in Table VII. Bearing weight losses are also given. With regard to the engine demerit ratings, it should be borne in mind that the lower the value is, the better the engine condition.

Table VII

| 40     | Oil                                                                                                                                                                                 | Engine demerits |           | Copper-lead connecting rod bearing weight loss |
|--------|-------------------------------------------------------------------------------------------------------------------------------------------------------------------------------------|-----------------|-----------|------------------------------------------------|
|        |                                                                                                                                                                                     | Valves          | Ring zone |                                                |
| 45 (A) | S. A. E. 30 base oil (35% extracted coastal +6% paraffinic) +0.324% barium bis-(diisobutyl phenoxy) sulfide +0.324% barium bis-(diisobutyl phenoxy) sulfide +0.162% stearyl alcohol | 2.00            | 3.45      | Milligrams 202                                 |
| 50 (B) | Oil A +0.25% tert.-butyl ether of ortho tert.-butyl p-cresol                                                                                                                        | 1.75            | 3.29      | 86                                             |

These results show that the ether additive not only reduced the corrosiveness of the compounded oil toward the alloy connecting rod bearings but also improved the detergent action of the oil as shown by the ring zone and valve condition of the engine.

**EXAMPLE 9**

Similar engine demerit tests were conducted for 168 hours in a Hercules Diesel engine at 1500 R. P. M., with an oil temperature of 210° F. and a water temperature of 180° F. The results are shown in Table VIII.

Table VIII

|     | Oil                                                                                                                                                                                 | Duration of test | Engine demerits |           |        |               | Bearing weight loss, 6 rods |                |
|-----|-------------------------------------------------------------------------------------------------------------------------------------------------------------------------------------|------------------|-----------------|-----------|--------|---------------|-----------------------------|----------------|
|     |                                                                                                                                                                                     |                  | Overall         | Ring zone | Sludge | Piston skirts |                             |                |
| (A) | S. A. E. 30 base oil (35% extracted coastal +6% paraffinic) +0.324% barium bis-(diisobutyl phenoxy) sulfide +0.324% barium bis-(diisobutyl phenoxy) sulfide +0.162% stearyl alcohol | Hours            | 84              | 2.50      | 3.18   | 1.35          | 4.17                        | Milligrams 466 |
|     |                                                                                                                                                                                     |                  | 168             | 3.81      | 4.11   | 1.73          | 4.42                        | 1,119          |
| (B) | Oil A +0.25% tert.-butyl ether of ortho tert.-butyl p-cresol                                                                                                                        |                  | 84              | 1.86      | 2.96   | 0.88          | 3.25                        | 165            |
|     |                                                                                                                                                                                     |                  | 168             | 2.03      | 3.66   | 1.42          | 4.08                        | 547            |

In this engine also the ether additive reduced the tendency of the compounded oil to corrode the bearings and improved the cleanliness of the engine. With the ether additive the engine condition was substantially no worse after 168 hours of operation than it was after only 84 hours of operation when the ether additive was not present.

EXAMPLE 10

Other engine tests were conducted with a C. F. R. single cylinder engine at 1800 R. P. M. for 60 hours, the oil temperature being 200° F. and the water temperature 200° F. The results are shown in Table IX.

Table IX

|     | Oil                                                                                                                          | Overall engine demerit |
|-----|------------------------------------------------------------------------------------------------------------------------------|------------------------|
| (A) | Base oil (35% paraffinic, S. A. E. 30+35% extracted coastal S. A. E. 80)                                                     | 1.68                   |
| (B) | Oil A+0.325% barium bis-(diisobutyl phenoxy) sulfide+0.325% barium bis-(diisobutyl phenoxy) disulfide+0.163% stearyl alcohol | 1.43                   |
| (C) | Oil B+0.25% tert.-butyl ether of ortho-tert.-butyl p-cresol                                                                  | 1.18                   |

Here again the ether additive markedly improved the engine performance of the compounded oil, the lower demerit rating indicating that the engine was in a much cleaner condition.

In addition to being employed in crankcase lubricants for Diesel and automotive engines, the additives of the present invention may also be used in light mineral oils such as spindle oils and textile oils, metal cutting oils, turbine oils, insulating and transformer oils, steam cylinder oils and greases. Also, since these additives achieve their detergent effect by modifying surface activity, their use in asphalt, road oils and waxes to improve wetting and adhesive properties is also contemplated. Likewise, they may be added to liquid fuels to increase their wetting ability for metals, enabling them to displace moisture which might otherwise cause corrosion of containers, fuel lines, pump parts, and the like.

This invention is not to be considered as limited by any theory as to the action of the various additives nor by any of the examples mentioned or described herein which are given for illustrative purposes only, but is to be limited solely by the terms of the appended claims.

We claim:

1. An organic composition containing a small quantity of an organic compound of the formula



where Ar is an aromatic nucleus, R is an organic radical, R' is a tertiary aliphatic radical and n is an integer, and a small quantity of an organic compound containing a salt-forming unit selected from the class consisting of metals and basic radicals and containing also the element sulfur, at least one atom of sulfur being in divalent form and linked directly to carbon or to an atom of sulfur which is linked to carbon.

2. An improved lubricant which comprises an oil base, a small quantity of a compound of the formula



where R is an organic radical, R' is a tertiary

aliphatic radical and n is an integer, and a small quantity of an organic compound containing a metal and the element sulfur, at least one atom of said sulfur being in divalent form and linked directly to carbon or to an atom of sulfur which is linked to carbon.

3. A lubricant for internal combustion engines which comprises a mineral oil base, a small quantity of an organic compound of the formula



where R and R' are aliphatic radicals and R'' is a tertiary aliphatic radical, and a small quantity of n organic compound containing a metal selected from groups I, II, III, IV, and VIII of the periodic table and containing also the element sulfur, at least one atom of sulfur being in divalent form and linked directly to carbon or to an atom of sulfur which is linked to carbon.

4. A lubricant for internal combustion engines which comprises a mineral oil base, a small quantity of the tertiary butyl ether of ortho-tertiary butyl p-cresol, and a small quantity of an organic compound containing a metal selected from groups I, II, III, IV, and VIII of the periodic table and containing also the element sulfur, at least one atom of sulfur being in divalent form and linked directly to carbon or to an atom of sulfur which is linked to carbon.

5. A lubricant for internal combustion engines which comprises a mineral oil base, a small quantity of an organic compound of the formula



where R and R' are selected from the group consisting of hydrogen and aliphatic radicals and R'' is a tertiary aliphatic radical, and a small quantity of a compound containing the radical



where M is a member of the group consisting of metals and basic radicals, X is a member of the group consisting of oxygen and sulfur and is attached to a carbon atom which is in turn attached only to atoms of the group consisting of hydrogen and other carbon atoms, R is a member of the group consisting of aliphatic and aromatic radicals, and n is an integer, one to four.

6. A lubricant for internal combustion engines which comprises a mineral oil base, a small quantity of an organic compound of the formula



where R and R' are selected from the group consisting of hydrogen and aliphatic radicals and R'' is a tertiary aliphatic radical, and a small quantity of a compound of the formula



in which M is a metal, X is a member of the group consisting of oxygen and sulfur, Ar is an aromatic nucleus, R is an organic group and n is an integer, one to four.

7. A lubricant for internal combustion engines which comprises a mineral oil base, a small quantity of the tertiary butyl ether of ortho tertiary butyl p-cresol and a small quantity of a salt of a metal of group II of the periodic table and a 5 phenoxy sulfide.

8. A lubricant for internal combustion engines which comprises a mineral oil base, a small quantity of the tertiary butyl ether of ortho tertiary butyl p-cresol and a small quantity of barium 10 bis-(diisobutyl phenoxy) sulfide.

9. A lubricant for internal combustion engines which comprises a mineral oil base, about 0.2% to about 2.0% of the tertiary butyl ether of ortho tertiary butyl p-cresol and about 0.02% to about 15 2.0% of barium bis-(diisobutyl phenoxy) sulfide.

10. A lubricant for internal combustion engines which comprises a mineral oil base, about 0.5% of barium bis-(diisobutyl phenoxy) sulfide, about 0.5% of barium bis-(diisobutyl phenoxy) disulfide, about 0.25% of stearyl alcohol and about 20 0.5% of the tertiary butyl ether of ortho tertiary butyl p-cresol.

11. A lubricant for internal combustion engines which comprises a mineral oil base, a small quantity of the tertiary butyl ether of ortho tertiary butyl p-cresol and a small quantity of zinc lauryl 25 mercaptide.

12. A lubricant for internal combustion engines which comprises a mineral oil base, a small quantity of the tertiary butyl ether of ortho tertiary butyl p-cresol and a small quantity of tin dicyclohexyl dithiocarbamate.

13. The method of cleansing and lubricating an internal combustion engine which consists in 30 charging the said engine and operating said engine with a lubricant comprising a mineral oil base, a small quantity of an organic compound 35 selected from the group consisting of metals and basic



where Ar is an aromatic nucleus, R is an organic radical, R' is a tertiary aliphatic radical and n is an integer, and a small quantity of an organic compound containing a salt-forming unit selected 40 from the class consisting of metals and basic

radicals and containing also the element sulfur, at least one atom of sulfur being in divalent form and linked directly to carbon or to an atom of sulfur which is linked to carbon.

14. The method of cleansing and lubricating an internal combustion engine which consists in charging to said engine and operating said engine with a lubricant comprising a mineral oil base stock, a small quantity of an organic compound of the formula



where R and R' are selected from the group consisting of hydrogen and aliphatic radicals and R'' is a tertiary alkyl radical, and a small quantity of an organic compound containing a metal selected from groups I, II, III, IV, and VIII of the periodic table and containing also the element sulfur, at least one atom of sulfur being in divalent form and linked directly to carbon or to an atom of sulfur which is linked to carbon.

15. The method of cleansing and lubricating an internal combustion engine which consists in charging to said engine and operating said engine with a lubricant comprising a mineral oil base, a small quantity of the tertiary butyl ether of ortho tertiary butyl p-cresol and a small quantity of barium bis-(diisobutyl phenoxy) sulfide.

16. A lubricant for internal combustion engines which comprises a mineral oil base, a small quantity of the tertiary butyl ether of ortho tertiary butyl p-cresol and a small quantity of a metal alkyl mercaptide.

17. A lubricant for internal combustion engines which comprises a mineral oil base, a small quantity of the tertiary butyl ether of ortho tertiary butyl p-cresol and a small quantity of a metal aliphatic dithiocarbamate.

JOHN G. McNAB.  
CARROLL J. WILSON.  
CARL WINNING.